

## UNITED STATES PATENT OFFICE.

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MASSACHUSETTS.

## HAIR FELT AND METHOD OF MAKING.

No Drawing.

Application filed September 12, 1923. Serial No. 662,221.

This invention has for its object to produce on a paper machine felt comprising a major portion of hair of original length. Such felt is adapted for a great variety of uses in the arts such as insulation against heat and sound, and as a basic material to be saturated with asphalt, bituminous materials, rosins, waxes or the like, or mixtures of these.

10 A difficulty found in the use of long hair in making felt on a paper machine is its strong tendency to become lumpy and matted in the furnish so that the formation on the cylinder mold, and the subsequent felting is not uniform, but the product has thick and thin portions and is improperly bonded. In order to break up these lumps, it has been necessary to set the beater roll down so hard that most of the hair was cut or broken 20 so that it has been relatively short in the final product.

I have discovered that such hard beating is not necessary if the hair be mixed with material which serves to lubricate and individualize it so that the strands thereof may slide by each other and become uniformly distributed in the stock. This may be accomplished by the use of a material of a slimy nature, such as a slimy soap, or 25 saponified oils or fatty acids, or combinations thereof. For example, 10 to 50 parts of cellulose fiber such as sulphate, or sulphite pulp, rags, cotton, linters, etc., or combinations thereof, are beaten out for about 30 fifteen minutes. The beater roll is then raised slightly so as to avoid cutting the hair but yet sufficiently down so as to comb out the hair, and from 50 to 90 parts of hair, such as goat or cattle hair from tanneries, 35 and about 20 parts of any ordinary soap solution are then added to the beater. This is circulated in the beater for about an hour, or until the hair is combed out and each fiber 40 is so coated with the soap as to be individualized. The mixture is then transferred to the wet machine and "run wet" or with a large volume of water, and with heavy suction on the cylinder mold. This method 45 in operating the machine helps to prevent the hair from becoming matted and aids in transferring the stock to the make-up roll 50 from the carrier felt. This produces a

somewhat rough surfaced felt of very open and porous nature but exceedingly tough when saturated.

55 Where the hair is individualized by such soap the soap may be washed out in the felting operation, thus leaving a distinctly open and porous product of no great strength when dry, if the amount of cellulosic material be very small, but when saturated, as with asphaltic or bituminous compounds, of great toughness and resistance to tearing and yet of great flexibility and elasticity so that it may be readily distorted and deformed and stretched without danger of tearing. Where a somewhat denser product is desired more cellulosic material 60 may be used, and also if desired, the soap may be precipitated after the individualizing has been effected, by adding alum to the mixture, the precipitate serving as a filler for the felt which causes it to be more dense and incapable of absorbing as large a proportion of the saturant. For certain 65 purposes, however, this denser and stronger felt may be highly desirable.

70 The function of the cellulosic material is more thoroughly to bond the hair, since this felts much more readily than the hair 75 and therefore aids in running the stock on the paper machine. The use of wood flour or sawdust also aids in this respect since it prevents the individualized hair fibers from slipping so easily relative to each other 80 so that they do not become so readily displaced after they have once been laid in the felting operation. Wood flour or sawdust alone, however, would not add materially 85 to the strength of the felted product, which when dry would be quite weak were the cellulosic fiber entirely omitted, and some fibrous cellulosic material has been found necessary in order that the stock may be 90 run satisfactorily on the paper machine.

95 Should the hair contain lime this would act to precipitate some of the soap in the felt which might or might not be desirable in individual instances, depending on the character of the felt desired.

100 By the expression "slimy soap" as used in the specification and appended claims, I mean the soap of a fatty acid, e. g., the sodium or potassium soap of oleic, stearic, or

palmitic acids, or the like, in contradistinction to sodium resinate or like soaps, which are of markedly less slimy or lubricating character.

- 5 It will thus be seen that the soaps which I employ and which are especially effective as individualizing agents are aliphatic or straight chain fatty-acids soaps, whereas sodium resinate, which is materially less 10 effective, falls in that class of soaps having an aromatic or ring structure.

Having thus described this invention it is evident that various changes and modifications will occur to those skilled in the 15 art such as properly come within the scope and spirit of the invention as defined by the appended claims.

I claim:

1. The method which comprises beating 20 together cellulosic material and soap having the slimy characteristics of a straight chain fatty-acid soap, then adding to the beater long hair and beating and combing out the fibers while maintaining them of original 25 length until they are thoroughly individualized, and then running off on a wet paper machine.

2. The method which comprises beating 30 together cellulosic material and soap having the slimy characteristics of a straight chain fatty-acid soap, then adding to the beater long hair, and beating and combing out the fibers while maintaining them of original 35 length until they are thoroughly individualized, and then running off on the paper machine with a large volume of water and under heavy suction.

3. The method which comprises beating 40 together cellulosic material and soap having the slimy characteristics of a straight chain fatty-acid soap, then adding long hair and beating and combing out the fibers while maintaining them of original length until 45 they are thoroughly individualized, precipitating the soap, and then running off on a paper machine.

4. The method which comprises individualizing hair of original length with soap

having the slimy characteristics of a straight chain fatty-acid soap, precipitating the soap 50 on the hair, and felting the stock.

5. The method which comprises individualizing hair of original length with soap having the slimy characteristics of a straight chain fatty-acid soap and felting the stock 55 on a wet paper machine.

6. A substantially uniform felt having the characteristics of paper machine fabrication and comprising animal and cellulosic fiber and an insoluble fatty-acid soap fixed thereon. 60

7. A substantially uniform felt having the characteristics of paper machine fabrication and comprising a preponderant proportion of long hair, a subordinate proportion 65 of cellulosic material, and an insoluble fatty-acid soap fixed thereon.

8. A substantially uniform felt having the characteristics of paper machine fabrication and comprising a preponderant proportion 70 of hair of substantially original length, a subordinate proportion of cellulosic material, and an insoluble fatty-acid soap fixed thereon.

9. A method which comprises individualizing with a soap having the slimy characteristics of a straight chain fatty-acid soap, the hair of a felt furnish comprising a preponderant proportion of hair of original length and a subordinate proportion of 75 cellulosic material, and felting the furnish on a wet paper machine.

10. A substantially uniform felt having the characteristics of paper machine fabrication and comprising 10 to 50 parts of 80 cellulose fiber, 50 to 90 parts of hair of original length and an insoluble fatty-acid soap fixed thereon.

11. A substantially uniform felt having the characteristics of paper machine fabrication and comprising hair, cellulose fiber, 85 sawdust, and an insoluble fatty-acid soap distributed therethrough.

In testimony whereof I have affixed my signature.

ALBERT L. CLAPP